

1  
2,701,815

## STABILIZED PHENYL-HYDRAZINE

Reinhard Böker and Hans Georg Fuchs, Frankfurt am Main, Germany, assignors to Farbwerke Hoechst Aktiengesellschaft vormals Meister Lucius & Brüning, Frankfurt am Main Hochst, Germany

No Drawing. Application October 27, 1953,  
Serial No. 388,656

Claims priority, application Germany October 29, 1952

### 5 Claims. (Cl. 260—569)

The present invention relates to stabilized phenyl-hydrazine.

The best and simplest characteristic for the determination of the degree of purity of phenyl-hydrazine is its solidification point, since already minute impurities result in a considerable drop of the solidification point of the phenyl-hydrazine. Pure phenyl-hydrazine which, for instance, is used in considerable quantities for carrying out syntheses on an industrial scale in the pharmaceutical industry, retains its theoretical solidification point of 19.6° C. only for a short period of time. It soon starts falling to reach only 11° C. after a 6 months' storage.

Now we have found that phenyl-hydrazine can be stabilized for a longer period of time by the addition of hexamethylene tetramine, preferably in proportions up to 3 per cent. strength. The addition of the said stabilizing agent may take place after the manufacture has been terminated or during the distillation for purity of the phenyl-hydrazine by adding dropwise a solution of hexamethylene tetramine saturated in the warmth.

Phenyl-hydrazine stabilized in this manner by the addition of hexamethylene tetramine of 2 per cent. strength has a solidification point of 19.3° C. and retains, even in the presence of metals which catalytically accelerate the decomposition, a solidification point of 19.3° C. to 18.1° C. (=100 per cent. to 98.5 per cent. of phenyl-hydrazine) for a period of more than 6 months at summer-like temperatures (25° C. to 35° C.) and a lighter shade, whereas non-stabilized phenyl-hydrazine turns slowly darker when being stored.

This stabilized product allows of a storage for a longer period of time which was hitherto impossible, and a shipping in metallic containers without substantial reduction of the percentage of phenyl-hydrazine. Furthermore, it is always advisable to dispatch stable phenyl-hydrazine if it is used as preliminary product for important syntheses of remedies.

The following example serves to illustrate the invention.

#### Example

In 500 grams of freshly distilled phenyl-hydrazine solidifying at 19.5° C. containing 99.5 per cent. of pure phenyl-hydrazine, there are dissolved 2 per cent. of hexa-

2

methylene tetramine; into the clear solution obtained a sheet of zinc is laid and the whole is allowed to stand at 25° C. to 35° C. in a closed, brown, glass-stoppered bottle. From time to time samples are taken from the bottle for the determination of the solidification point and the degree of purity of the phenyl-hydrazine, the results obtained being compared with samples of non-stabilized phenyl-hydrazine subjected to the same conditions.

The following table indicates the solidification points and degrees of purity of the two samples depending on the time of storage.

| 15 | Time (months) | Phenyl-hydrazine non-stabilized |                 | Phenyl-hydrazine stabilized |                 |
|----|---------------|---------------------------------|-----------------|-----------------------------|-----------------|
|    |               | Solidification Point            | Content Percent | Solidification Point        | Content Percent |
| 20 | 0             | 19.5                            | 99.5            | 19.3                        | 99.5            |
|    | 1             | 18.5                            | 98.5            | 19.0                        | 99.3            |
|    | 2             | 16.7                            | 97.3            | 18.9                        | 99.0            |
|    | 3             | 14.5                            | 95.7            | 18.8                        | 98.9            |
|    | 4             | 14.3                            | 94.4            | 18.7                        | 98.7            |
|    | 5             | 12.5                            | 93.2            | 18.4                        | 98.6            |
|    | 6             | 11.0                            | 91.7            | 18.1                        | 98.5            |
|    | 7             | 10.1                            | 89.5            | 18.0                        | 98.5            |

After a 7 months' storage under closure the non-stabilized material sustained a loss of about 10 per cent. of its efficacy, whereas the stabilized material sustained a loss of about 1 per cent. under the same conditions. The rapidity of decomposition of the stabilized material after a 7 months' storage has thus been reduced to about one tenth of that of the non-stabilized product. At an increased access of air as well as at elevated temperatures an even greater difference is to be expected.

After a 12 months' storage under exclusion of air, stabilized phenyl-hydrazine still has a degree of purity of 96.1 per cent. solidifying at 17.3° C., whereas the non-stabilized product contains only 65.7 per cent. of phenyl-hydrazine.

We claim:

1. A stable phenyl-hydrazine, wherein hexamethylene tetramine is present in a proportion of 1 to 3 per cent.
2. A stable phenyl-hydrazine, wherein hexamethylene tetramine is present in a proportion of about 2 per cent.
3. A process for the manufacture of a stable phenyl-hydrazine, comprising addition of hexamethylene tetramine in a proportion of 1 to 3 per cent. to phenyl-hydrazine.
4. A process for the manufacture of a stable phenyl-hydrazine, comprising addition of hexamethylene tetramine in a proportion of 1 to 3 per cent. during the distillation for purity of phenyl-hydrazine.
5. A process for the manufacture of a stable phenyl-hydrazine, comprising addition of hexamethylene tetramine in a proportion of 1 to 3 per cent. after the manufacture of phenyl-hydrazine.

No references cited.